

## UNITED STATES PATENT OFFICE

2,363,001

## NONVOLATILE HYDROCARBON PRODUCTS

Everett C. Hughes, Cleveland Heights, Ohio, assignor to The Standard Oil Company, Cleveland, Ohio, a corporation of Ohio

No Drawing. Application November 11, 1943,  
Serial No. 509,899

6 Claims. (Cl. 252—49)

It has become a custom in the industry to designate as "anti-oxidants" or oxidation inhibitors agents which exert an effect of preventing deterioration in hydrocarbon products. Irrespective of any questions of accuracy of such designation, the convenience of the term has led to a quite general acceptance, and the practical effect of such agents is quite generally recognized. In accordance with the present invention, certain improvements along such lines are now made possible, and involving materials which are available without undue cost.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The hydrocarbon product, such as an oil, asphalt, etc., is, in accordance with the invention, subjected to the action, in service, of a soluble sulphide of phosphorus having a lower sulphur content than  $P_2S_5$ , in a small amount. Sulphides of this character are  $P_4S_2$ ,  $P_2S_3$ ,  $P_3S_6$ ,  $P_4S_3$ ,  $P_4S_5$  being particularly desirable. The amount of such phosphorus sub sulphide may be 0.001-2%, and usually 0.01-0.05%. Where the mineral oil is of lubricating character, lubricating viscosities may be as desired, or for instance 45-200 sec. Saybolt Universal at 210° F. Peculiarly, I have found that by adding also another agent which is an oxidation inhibitor, the total effect of the combination is out of proportion to the additive action merely of the phosphorus sulphide and the other inhibitor, and presents unique advantages; and besides, there is a lessened tendency to metal corrosion, a matter which is desirable in some usages.

Such additional inhibitor may be for instance an amino diphenyl methane derivative, as di-amino diphenyl methane, tetramethyl diamino diphenyl methane, Michler's hydrol or  $pp'$   $(CH_3CH_2N)_2(C_6H_5)_2CHOH$ , tetramethylene pentamine, diphenylamine, alpha naphthylamine, beta naphthylamine, quinoline, brucine, acetooacetanilide, lecithin, nitrobenzene, nitrotoluene, and such nitrogen containing organic compounds. Where treating a normally solid hydrocarbon product such as asphalt to prevent its deterioration or so-called "oxidation change" in service, the addition agents are introduced with the asphalt in molten condition. Mineral oils

containing the phosphorus sulphides as noted, with or without another inhibitor, also have excellent extreme pressure lubricating action. The amount of said additional nitrogen containing inhibitor preferred for use in connection with the above defined sulphide of phosphorus is within the range of 0.1 to 1.0%. However, amounts as low at 0.001% give substantial improvements and amounts this low therefore may be used. In general it is not economic to use more than 5%.

As an example: To a 20 S. A. E. lubricating stock of Mid-Continent origin there is added 0.05% of  $P_4S_3$  and 0.25% of tetramethyldiamino-diphenylmethane. This lubricant, as tested by subjecting to the bubbling through of air at the rate of 30 liters of air per hour for 65 hours at 300° F., showed a viscosity increase at 100° F. of 20, naphtha insolubles 0.8%, lacquer formation 6.8, and appearance rating B-. In contrast, the same oil without the addition agents, similarly tested, showed a viscosity increase of 247, naphtha insolubles 9.8%, lacquer formation 40.5, and appearance rating D.

As another example: In a similar oil there is incorporated 0.05% of  $P_4S_3$  and 0.25% of di-amino diphenylmethane. This lubricant when tested as foregoing, showed viscosity increase of 27, naphtha insolubles 0.8%, lacquer formation 8.3, and appearance rating C+.

As another example: In a similar oil there is incorporated 0.05%  $P_4S_3$  and 0.13% of Michler's hydrol. This lubricant, when similarly tested as the foregoing, showed a viscosity increase of 20, 0.6% of naphtha insolubles, lacquer formation 6.0, and appearance rating B+.

This application is a continuation-in-part of my application Serial Number 332,617, filed April 30, 1940.

I claim:

1. A normally non-volatile hydrocarbon product containing  $P_4S_3$  in effective amount up to 2 per cent to stabilize against oxidation, and including also 0.25 per cent of an amino diphenyl methane derivative.

2. A normally non-volatile hydrocarbon product containing  $P_4S_3$  in effective amount up to 2 per cent to stabilize against oxidation, and including also 0.25 per cent of diaminodiphenylmethane.

3. A normally non-volatile hydrocarbon product containing  $P_4S_3$  in effective amount up to 2 per cent to stabilize against oxidation, and including 0.13 per cent of Michler's hydrol.

4. A normally non-volatile hydrocarbon prod-

uct containing  $P_4S_3$  in effective amount up to 2 per cent to stabilize against oxidation, and including 0.001% to 5% of an amino diphenyl methane derivative.

5. A normally non-volatile hydrocarbon product containing  $P_4S_3$  in effective amount up to 2 per cent to stabilize against oxidation, and including 0.001% to 5% of a nitrogen containing oxidation inhibitor.

6. A normally non-volatile hydrocarbon product containing a sulphide of phosphorus having a lower sulphur content than  $P_2S_3$  in effective amount up to 2 per cent to stabilize against oxidation, and including 0.001% to 5% of a nitrogen containing oxidation inhibitor.

EVERETT C. HUGHES.